

B. T. COLLEY,  
SMELTING AND BRIQUETING PROCESS,  
APPLICATION FILED DEC. 15, 1911.

1,098,883.

Patented June 2, 1914.



# UNITED STATES PATENT OFFICE.

BERNARD T. COLLEY, OF RANCAGUA, CHILE.

## SMELTING AND BRIQUETING PROCESS.

1,098,883.

Specification of Letters Patent. Patented June 2, 1914.

Application filed December 15, 1911. Serial No. 665,878.

To all whom it may concern:

Be it known that I, BERNARD T. COLLEY, a subject of the King of Great Britain, residing at Rancagua, Republic of Chile, have 5 invented certain new and useful Improvements in Smelting and Briquetting Processes, of which the following is a specification.

This invention deals with various improvements in the metallurgical treatment 10 of mineral-bearing materials; and from one aspect it involves a preliminary treatment whereby certain ores which have heretofore been better suited for reverberatory-furnace work may now be briqueted with various 15 binders for blast-furnace smelting; from another aspect it is concerned with the formation of briquets from a new combination of ingredients including "briquet roasted" ores with my novel binding-agent; from another 20 aspect it combines and inter-relates either or both of these improvements with certain other economic adaptations of the general smelting system. It is noteworthy however that certain advantages characteristic 25 of a somewhat specific but very valuable embodiment of this invention prominently appear in its utilization whereby ordinary "fines" may be briqueted through the instrumentality of plaster of Paris as a binding agent in combination with the other ingredients of the briquet.

One object within the contemplation of this invention is to simplify the smelting of sulfur-bearing ores available in a committed 30 condition by means of a process in which certain steps will be so formulated individually and will be so related to other operations that the major difficulties ordinarily encountered in customary methods of 35 treating such ores from a commercial standpoint will be largely obviated or practically eliminated.

Another object is to make it commercially possible to satisfactorily briquet certain ores, 40 which for reasons heretofore obscure have resisted efforts in that direction, by ascertaining the real causes and proposing a remedy whereby such ores may be brought into a condition suitable for briquetting.

50 A further object of this invention is to devise a system of briquetting such that raw materials readily available *in situ* may, in connection with certain parts of the general process be well adapted for use as a binder in 55 the briquetting operation.

A further object is to devise a binder of a character readily available in commerce or capable of being manufactured in a simple and inexpensive manner at the smelter by utilizing certain waste products thereof, and 60 which will be of a nature capable of being readily handled by unskilled labor in briquetting fine ore concentrates without requiring the use of slow-operating and involved machines employing high pressures 65 in the molding; but which binder may easily be made into bricks with ores through the instrumentality of simple brickmaking machines requiring a minimum of time and attendance.

This invention furthermore proposes a binder which will act in a very effective manner to hold particles of the briquet together even when stored during long intervals of time or when subjected to relatively 70 rough handling and which will operate satisfactorily in a blast furnace.

Another and still more specific aim of this invention is to provide a binder consisting of sulfur bearing material which when used as 80 proposed for briquetting sulfur-bearing ores will be of a very permanent character and avoid or effectively resist the disintegrating influences to which other binders have yielded during a period of storage or while handling the same.

The annexed drawing diagrammatically illustrates a general smelting and briquetting system exemplifying the various features of 85 this invention and the cyclic relation therebetween.

As an introductory to a more detailed discussion of the novel features underlying the commercial utility of this invention, it may be preliminarily observed that the extraction 90 of metals from their ores, as, for example, copper from its sulfur-bearing concentrates, consists of a number of successive steps or treatments all of which are more or less interdependent. A difficulty frequently encountered in one of these steps resides in the handling of finely divided ore concentrates in the blast furnace. To satisfactorily operate a blast furnace, the charge should be composed of comparatively large lumps, because fine ores are the occasion of heavy mechanical losses when smelting in the blast-furnace. For that reason, in copper smelting, a reverberatory furnace is now very generally used for fine ores.

To devise a method of briquetting which will be altogether simple from a manipulative standpoint and equally effective from a metallurgical standpoint, while at the same time obviating the difficulties encountered in current practice, has been the goal for which those most skilled in this art have long striven. Many methods for preparing fine ores for blast-furnace smelting have been proposed and tested with only mediocre success either because no adequate binder has been recognized as yet with which briquets of sufficient consistency or resistancy could be made or it has not been discerned heretofore that by a certain treatment the ores may be so changed in condition as to satisfy the requirements of the binder and obviate the difficulty. So also, certain otherwise available binding agents have been discarded or escaped the selective attention of the metallurgist by reason either of their commercial nonavailability in remote quarters or because of an inability to devise a method of locally manufacturing such agents which, in a manner essentially harmonious with the general smelting operations, will utilize certain otherwise waste products thereof, and thus introduce economies.

By this invention, however, I have not only specifically improved the art of briquetting by utilizing plaster of Paris as a binding agent in combination with the other ingredients, but I have also formulated an improvement in the general smelting scheme whereby various ores which have heretofore failed to respond to briquetting are rendered highly available by a very inexpensive treatment and whereby certain other operations may be carried out in a way and to an extent not heretofore commercially possible. I have also so devised the general scheme of smelting that the binding agent, plaster of Paris, preferably employed in the briquetting step may be produced economically through the instrumentality of other steps, such as a roasting operation, thus utilizing waste products, such as sulfur-bearing gases and at the same time materially reducing the emission of such gases into the atmosphere of the neighboring community.

It has been observed heretofore that briquets made of certain classes of ores under prevailing methods are unsatisfactory owing to the fact that they disintegrate prematurely in the blast-furnace. The cause of the failure has been attributed to the effect of pressure and an incompatibility between the binding agent and the particular ore used under the conditions in the furnace or otherwise. I have, however, discovered as a result of extensive investigations that two very potent factors, either or both of which may cause the failures, are: (a) an intensified capacity for deflagrating possessed by cer-

tain materials, and (b) the presence in certain ores of compounds such as  $FeS_2$  which evolve sulfur at low temperatures, and I have further ascertained that these factors may be sufficiently eliminated by an inexpensive preliminary step in the briquetting process, so that all such ores may be briquetted and efficiently smelted in the blast-furnace even by utilizing binding-agents previously incapable of satisfactory service, but preferably my new combination of mineral-bearing materials with my proposed binding-agent should be used if the highest efficiency is sought for. Nearly all ores, including sulfids, deflagrate more or less, and all sulfid ores containing  $FeS_2$  break at red-heat. In the furnace, this would give rise to flue-dust and other difficulties encountered in blast furnace practice where fine ore exists. Materials, free from  $FeS_2$ , may deflagrate quite violently, but if also free from the deflagrating substance may be successfully briquetted like an ordinary matte.

To convert materials in a physical or chemical state antagonistic to briquetting to a condition compatible under furnace conditions with the cementing properties of the binder used, this invention proposes what may be termed a "briquetting roast" as a preparatory step in the briquetting process. This step involves a preliminary heating to a dull-red heat or thereabout for a suitable period, say for fifteen minutes or more, preferably under controlled access of air, whereby the atom of sulfur may be driven off of such  $FeS_2$  as may be present and whereby the deflagrating material present is also disintegrated or broken down to an extent such that no further rupture of consequence takes place prematurely. This preliminary heating or roasting to adapt the ores for briquetting is believed to be without precedent and is to be distinguished from an ordinary roasting operation performed for other purposes. The particular apparatus employed for this operation is not of the essence of this aspect of my invention, since any type of roaster may be used, but, since I also propose to stop the further rise in temperature and prevent a further loss of sulfur combined as  $FeS$ ,  $Cu_2S$ , etc. when the material treated has reached the necessary degree of temperature, I prefer to use an apparatus permitting a very good control of the air admitted, such as the MacDougal, Herresshoff or Wedge roasters. Should fuel be needed, any kind may be used, but since the roasting or heating period will be short, the fuel consumption will be very small if not entirely negligible, especially since the heat wasted in flues (as from a converter) could be utilized.

Unless first eliminated, as above indicated, the atom of sulfur set free when the  $FeS_2$  is reduced would in its escape cause a

briquet to weaken, open and break when it reached the dull red zone of the furnace. Its initial elimination from the briquet should not be regarded as a metallurgical loss, however, for, since in any event it would be expelled at a dull red heat without oxidation, it would neither be available for matte formation nor valuable as a fuel since it does not generate heat. On the other hand, owing to the excellence of briquets made from pre-treated ore, especially with my new binding agent, my system will more thoroughly realize the advantages of the sulfur combined as FeS since more of a given proportion of sulfur may be carried unaltered to the fusion-zone, permitting less fuel or faster driving so that, even with a normal ore charge, it may be advisable to screen and briquet the fines in accordance with my system, since even with the normal charge there can be little doubt that the utility of the sulfur as FeS is diminished by fine breakage and premature oxidation. In my preliminary "briquet-roast," the complete elimination of the extra atom of sulfur may also be attended with the oxidation of from 1% to 3% of the sulfur combined as FeS, and the fuel value of this sulfur will correspondingly reduce or even entirely obviate the need for extraneous fuel, since its heat may suffice to maintain the required temperature. Irrespective of this, however, my system, as above stated, enables a greater percentage of the sulfur of the FeS to actually reach the fusion zone and become metallurgically available as a smelting agent.

It has been determined that briquets made by this process from many kinds of ores, concentrates, etc., have uniformly given excellent results in smelting tests. Throughout the temperature changes from cold to the heat of incipient fusion, they have given no signs of breakage though sustaining pressures up to 10 lbs. per. sq. in. during a period of about 4 hrs. From observations, they appear to gradually subside while still retaining their original form as the fusion takes place, until the mass is so softened that it becomes quite plastic throughout and yields to the pressures.

The value of my "briquetting roast" is accentuated in connection with my new binding agent (plaster of Paris), but the preliminary treatment is also of great utility when inferior binders are used, such as lime, clay, slimes, etc., and such treatment in that relation is therefore comprehended by one aspect of my invention.

A suitable starting material, from which my new briquetting binder may be made, is ordinary lime-stone which is, of course, readily available to all smelters. This invention proposes as a useful sub-process to transform this lime-stone into plaster of Paris, preferably by methods more or less

dependent upon certain steps in the general smelting process. Here it may be noted that since smelters usually use a very pure grade of limestone, the resultant plaster of Paris will be white and therefore well suitable for general sale. The gases from the furnace roasters or converters contain considerable proportions of sulfur dioxid and this may be converted into sulfuric acid by well known methods and the crushed limestone may then be converted into hydrated calcium sulfate by dissolving the same in this more or less diluted sulfuric acid. The manufacture of the acid can be done most cheaply by means of a tower of the Glover type and by catalytic action, and sufficient  $\text{SO}_3$  can be obtained from converter gases by controlling the amount of air admitted to the flue, especially if such converter is of the Pierce-Smith type, which will treat matter containing 22% sulfur. Again, the Cotrell process may be resorted to in this connection and would possess the advantage of collecting the values otherwise lost in the gases.

I have made tests on the efficiency of the conversion of the limestone into hydrated calcium sulfate by dissolving the stone crushed into various sizes ranging from 100 mesh progressively through 30 mesh, 20 mesh, 10 mesh, pea, bean and walnut sizes. As the result of such experiment, I have ascertained that 10 mesh or 20 mesh would be serviceable even without stirring, but with the aid of mechanical stirring even coarser sizes could be used, as the calcium sulfate would be flaked away from the nucleus to expose fresh surfaces of the limestone to the action of the acid. This operation will preferably be carried out in a lead lined vat with a stirring paddle actuated mechanically. I have also ascertained that solutions of acid as low as 20 per cent.  $\text{H}_2\text{SO}_4$  work efficiently and when all the carbonate has been transferred into the hydrated calcium sulfate, the entire charge is run out of the acid treatment vat either into a washing vat or through a filter press. A washing vat may be used since the calcium sulfate is of sufficient body to permit of washing in flat tanks by slow-running water, but I prefer to use a filter press and concomitantly gain the advantage of reducing the percentage of moisture to the lowest point, so that the cost of dehydration (if not effected by waste heat) may be as low as possible. The product thus obtained is a more or less moist sludge of hydrated calcium sulfate which (assuming 30 per cent. free water and 10 per cent. of water of crystallization) will require a treatment for some hours at a temperature not higher than 120 degrees C. in order to effect an evaporation of the free water and also drive off one-half of the water of crystallization. This may be ac-

complished by steam maintained at a suitable pressure, but it is however, perfectly feasible to utilize the waste heat from the converter to dehydrate the gypsum. This 5 possesses the advantage that the gases which enter the mouth of the flue from the converter at 1000 degrees C., would be cooled by the endothermic dehydration process to a temperature below the formation point of 10  $\text{SO}_3$  i. e. 430 degrees. Therefore, these sulfur-bearing gases may be simultaneously utilized by a proper exclusion of air from the flue, for the dehydration and the production of the acid. The temperature may be 15 maintained at 120° C. in the dehydrating vats in various ways, as by the use of steam or automatic temperature controllers which would bypass the gases. Temperature variations below 120° C. resulting from converter fluctuations may occur without an undue interference with the dehydration process, since the latter can take place at a temperature as low as 80°, but the temperature should not rise above 120° C., otherwise the 20 other molecule of water will be driven off. It is noteworthy in this connection that the plaster of Paris as thus produced needs no crushing and can be used as drawn from the dehydrating pans, and if the dust has been 25 kept from the acid-making gases and a good grade of limestone has been employed, the product will be quite pure and white and well suited for the ordinary applications of this cement. Thus, I have proposed a novel 30 and essentially practicable method of producing plaster of Paris commercially. By thus lessening the cost of this cement, it may now be used where heretofore prohibited, for even with coarse particles it makes a 35 good strong concrete well suitable for many purposes.

A very important embodiment of an integral part of my invention is based on my discovery that briquets in which plaster of 45 Paris is used as the binding agent are remarkable for their excellence from a metallurgical standpoint. I have ascertained as a result of my experiments that, when ore is briqueted with even smaller percentages of 50 plaster of Paris than is customary with other binders, the briquets possess very superior qualities in hardness and sustaining power.

An advantage promoting rapid production and handling resides in the fact that my binder comes quickly to a good set. I have also discovered that it is not essential or materially advantageous to employ pressures in forming the briquets, and consequently the operation may be performed by 55 means of a wire-cut brick-machine thereby materially lowering the cost of briquetting as compared with machines of the pressure type. Preferably, a machine will be used 60 which will perform its work within two

minutes from the time the material is wetted and fed to the machine. From 5-10% of plaster of Paris is recommended for ordinary cases, and generally about 5% will suffice, and coarser particles of materials may 70 be handled as easily as "fines" because my binder acts very much as does the cement in concrete.

The plaster of Paris may be employed for briqueting sulfur-bearing ores with great 75 advantage and such bricks may be stored for long periods without disintegrating, by the oxidation of sulfids into sulfates or by similar chemical reactions such as could occur with other cements, owing to the fact that 80 plaster of Paris is itself a sulfate compound. Within ten minutes or less, the briquets thus made will take a comparatively firm set, and consequently, my system does not require the exercise of extraordinary care in handling the same to prevent breakage, and with proper provisions to avoid excessive falls, much of the labor and pains heretofore necessary with other binders may be avoided by using a belt for delivering the briquets 85 directly to the bins. The firmness, durability and thorough effectiveness of the briquets thus made will appeal at once to any metallurgist, especially in the light of the applications thereof herein proposed. I 90 have thus made without pressure briquets of copper concentrates with 5% of my binder, which after three days sustained a pressure of upward of 90 lbs. per square inch, as against 45 lbs. per square inch sustained by briquets similarly made with burnt lime as the binder. I have also discovered that, contrary to what might be expected, my briquets do not appear to crumble or break by the dehydration of the calcium-sulfate when heating to fusion, but appear to possess the remarkable quality of 95 retaining their shape while melting until complete fusion. Thus, my briquets should reach the fusion-zone of a smelting-furnace 100 without breakage or dust loss.

This invention proposes by the utilization of my system of briqueting to effect certain economic changes in current methods of smelting. Thus, whenever 20% of 105 the sulfur content of a blast-furnace charge does not exceed the copper content by sufficient quantity to produce a matte too low for economic converting, then roasting is not only unnecessary but detrimental, because all the iron and sulfur oxidized during the smelting operation have a large fuel value. Under these circumstances, I therefore propose to replace sintering by the plaster briquets which will allow all the sulfur and iron to be oxidized directly in the blast-furnace, thereby avoiding the use of a material calling for reduction and necessitating a corresponding increase in the fuel expenditure.

My method of briquetting and my new briquets will enable a blast-furnace operation to be adopted for a charge composed entirely of concentrates, and thus replace the reverberatory furnace which has always been used under such conditions. Furthermore, my system could be advantageously used in connection with a charge prepared for lead-smelting for fine ores not requiring to be roasted, since the sulfur of the binder would be driven off as  $\text{SO}_3$  and would not enter into the formation of matte. In plants which depend on concentrates for their supply of sulfur, this system would also be very advantageous as the briquet being hard and compact would deliver the sulfur into the fusion zone much as does lumpy ore.

Viewing the foregoing, in the light of current knowledge those skilled in this art will thereafter be enabled to readily utilize various steps and relations thereof which shall have become known as interchangeably available with and metallurgically equivalent to those herein specified and which, although perhaps calculated to appear widely different under a superficial inspection, and follow in a varied sequence, would nevertheless embody certain if not all of the herein described features which, from the aspect of the prior art, constitute essential and advantageous characteristics of this invention, and therefore such processes should and accordingly are intended to be comprehended within the wording and scope of the following claims.

Having thus disclosed my invention through the foregoing typical examples thereof, I claim as new and desire to secure by Letters Patent:

1. A method of briquetting materials containing or composed of a substance having the capacity of evolving sulfur at a dull-red heat comprising heating the material at a dull-red heat or over for a short time, mixing the pre-treated material with a suitable quantity of a binding-agent, and then forming the resultant mixture into a multiplicity of blocks.

2. A method of briquetting materials containing  $\text{FeS}_2$  comprising heating the material for a short period at about a dull-red temperature to convert the  $\text{FeS}_2$  into  $\text{FeS}$ , mixing the pre-treated material with a suitable quantity of a binding-agent, and then forming the resultant mixture into a multiplicity of blocks.

3. A method of briquetting materials containing or composed of a deflagrating substance comprising heating the material at about a dull-red or upward for a short period, mixing said pre-treated material with a suitable quantity of a binding agent, and then forming the resultant mixture into a multiplicity of blocks.

4. A method of briquetting materials containing or composed of a substance having the capacity of deflagrating below smelting temperature comprising heating the material at the deflagrating temperature until the deflagrating action has substantially ceased, mixing said pre-treated material with a suitable quantity of a binding agent, and then forming the resultant mixture into a multiplicity of blocks.

5. A method of briquetting materials containing or composed of a substance having the capacity of evolving gaseous matter below smelting temperatures comprising heating the material at its gas-evolving temperature until the evolution has substantially discontinued, mixing said pre-treated material with a suitable quantity of a binding agent, and then forming the resultant mixture into a multiplicity of blocks.

6. A method of briquetting materials containing or composed of a substance having the capacity of evolving sulfur below smelting temperatures comprising heating the material at its sulfur evolving temperature until the evolution has substantially discontinued, mixing the pre-treated material with a suitable quantity of a binding agent, and then forming the resultant mixture into a multiplicity of blocks.

7. A method of briquetting materials containing or composed of deflagrating substance comprising heating the material at about a dull-red or upward for a short period, mixing said pre-treated material with a suitable quantity of plaster of Paris and then forming the resultant mixture into a multiplicity of blocks.

8. A method of briquetting materials containing or composed of a substance having the capacity of deflagrating below smelting temperatures comprising heating the material at the deflagrating temperature until the deflagrating action has substantially ceased, mixing said pre-treated material with a suitable quantity of plaster of Paris and then forming the resultant mixture into a multiplicity of blocks.

9. A method of briquetting materials containing or composed of a substance having the capacity of evolving gaseous matter below smelting temperatures comprising heating the material at its gas-evolving temperature until the evolution has substantially discontinued, mixing said pre-treated material with a suitable quantity of plaster of Paris and then forming the resultant mixture into a multiplicity of blocks.

10. A method of briquetting materials containing or composed of a substance having the capacity of evolving sulfur below smelting temperatures comprising heating the material at its sulfur evolving temperature until the evolution has substantially discontinued, mixing the pre-treated material

- with a suitable quantity of plaster of Paris, and then forming the resultant mixture into a multiplicity of blocks.
11. A method of briqueting materials containing or composed of a substance having the capacity of evolving sulfur at a dull-red heat comprising heating the material at a dull-red heat or over for a short time, mixing the pre-treated material with a suitable quantity of plaster of Paris and then forming the resultant mixture into a multiplicity of blocks.
12. A method of briqueting materials containing  $FeS_2$  comprising heating the material for a short period at about a dull-red temperature to convert the  $FeS_2$  into  $FeS$ , mixing the pre-treated material with a suitable quantity of plaster of Paris and then forming the resultant mixture into a multiplicity of blocks.
13. A method of briqueting mineral sulfids containing or composed of a deflagrating substance comprising heating the material at about a dull-red or upward for a short period, mixing said pre-treated material with a suitable quantity of plaster of Paris and water and then forming the resultant mixture into a multiplicity of blocks.
14. A method of briqueting concentrates containing or composed of a substance having the capacity of deflagrating below smelting temperatures comprising heating the material at the deflagrating temperature until the deflagrating action has substantially ceased, mixing said pre-treated material with a suitable quantity of water and plaster of Paris and then promptly forming the resultant mixture while in a plastic state into a multiplicity of blocks.
15. A method of briqueting concentrates containing or composed of a substance having the capacity of evolving gaseous matter below smelting temperatures comprising heating the material at its gas-evolving temperature until the evolution has substantially discontinued, mixing said pre-treated material with a suitable quantity of water and plaster of Paris and then forming the resultant mixture into a multiplicity of blocks.
16. A method of briqueting mineral sulfids containing or composed of a substance having the capacity of evolving sulfur below smelting temperatures comprising heating the material at its sulfur evolving temperature until the evolution has substantially discontinued, mixing the pre-treated material with a suitable quantity of water and plaster of Paris and then forming the resultant mixture into a multiplicity of blocks.
17. A method of briqueting mineral sulfids containing or composed of a substance having the capacity of evolving sulfur at a dull-red heat comprising heating the material at a dull-red heat or over for a short time, mixing the pre-treated material with water and about 5 to 10% of plaster of Paris, and then forming the resultant moist mixture into a multiplicity of blocks.
18. A method of briqueting concentrates containing  $FeS_2$  comprising heating the material for a short period at about a dull-red temperature to convert the  $FeS_2$  into  $FeS$ , mixing the pre-treated material with a suitable quantity of water and plaster of Paris, and then forming the resultant mixture into a multiplicity of blocks.
19. A method of briqueting sulfur-bearing materials containing or composed of a deflagrating substance comprising heating the material at about a dull-red or upward for a short period, mixing said pre-treated material with water and about 5 to 10% of plaster of Paris, and then forming the resultant moist mixture into a multiplicity of blocks.
20. A method of briqueting sulfur-bearing materials containing or composed of a substance having the capacity of deflagrating below smelting temperatures comprising heating the material at the deflagrating temperature until the deflagrating action has substantially ceased, mixing said pre-treated material with water and about 5 to 10% of plaster of Paris, and then forming the resultant moist mixture into a multiplicity of blocks.
21. A method of briqueting sulfur-bearing materials containing or composed of a substance having the capacity of evolving gaseous matter below smelting temperatures comprising heating the material at its gas-evolving temperature until the evolution has substantially discontinued, mixing said pre-treated material with water and about 5 to 10% of plaster of Paris, and then forming the resultant moist mixture into a multiplicity of blocks.
22. A method of briqueting concentrates containing or composed of a substance having the capacity of evolving sulfur below smelting temperatures comprising heating the material at its sulfur evolving temperature until the evolution has substantially discontinued, mixing the pre-treated material with water and about 5 to 10% of plaster of Paris, and then forming the resultant moist mixture into a multiplicity of blocks.
23. A method of briqueting concentrates containing or composed of a substance having the capacity of evolving sulfur at a dull-red heat comprising heating the material at a dull-red heat or over for a short time, mixing the pre-treated material with water and about 5 to 10% of plaster of Paris, and then forming the resultant moist mixture into a multiplicity of blocks.

24. A method of briquetting mineral sulfids containing  $FeS_2$ , comprising heating the material for a short period at about a dull-red temperature to convert the  $FeS_2$  into  $FeS$ , mixing the pre-treated material with water and about 5 to 10% of plaster of Paris, and then forming the resultant moist mixture into a multiplicity of blocks. 5 and permitting the same to set prior to using the same.
25. A method of briquetting of the nature disclosed consisting in mixing comminuted ore with a relatively small amount of a hydratable sulfur-bearing cementitious material and then promptly forming the resultant mixture while in a plastic state into a multiplicity of blocks, and permitting the same to set prior to using the same. 10
26. A method of briquetting of the nature disclosed consisting in mixing sulfur-bearing fines with a relatively small amount of a hydratable sulfur-bearing cementitious material and then promptly forming the resultant mixture while in a plastic state into a multiplicity of blocks, and permitting the same to set prior to using the same. 15
27. A method of briquetting of the nature disclosed consisting in mixing a charge composed entirely of concentrates with a relatively small amount of a hydratable sulfur-bearing cementitious material and then promptly forming the resultant mixture while in a plastic state into a multiplicity of blocks, and permitting the same to set prior to using the same. 20
28. A method of briquetting of the nature disclosed consisting in mixing copper and sulfur-bearing fines with a relatively small amount of a hydratable sulfur-bearing cementitious material and then promptly forming the resultant mixture while in a plastic state into a multiplicity of blocks, and permitting the same to set prior to using the same. 25
29. A method of briquetting of the nature disclosed consisting in mixing comminuted ore with about 5-10% of a hydratable sulfur-bearing cementitious material and then promptly forming the resultant mixture while in a plastic state into a multiplicity of blocks, and permitting the same to set prior to using the same. 30
30. A method of briquetting of the nature disclosed consisting in mixing sulfur-bearing fines with about 5-10% of a hydratable sulfur-bearing cementitious material and then promptly forming the resultant mixture while in a plastic state into a multiplicity of blocks, and permitting the same to set prior to using the same. 35
31. A method of briquetting of the nature disclosed consisting in mixing a charge composed entirely of concentrates with about 5-10% of a hydratable sulfur-bearing cementitious material and then promptly forming the resultant mixture while in a plastic state into a multiplicity of blocks, and permitting the same to set prior to using the same. 40
32. A method of briquetting of the nature disclosed consisting in mixing copper and sulfur-bearing fines with about 5-10% of a hydratable sulfur-bearing cementitious material, and then promptly forming the resultant mixture while in a plastic state into a multiplicity of blocks, and permitting the same to set prior to using the same. 45
33. A method of briquetting of the nature disclosed consisting in mixing comminuted ore with about 5-10% of plaster of Paris and then promptly forming the resultant mixture while in a plastic state into a multiplicity of blocks, and permitting the same to set prior to using the same. 50
34. A method of briquetting of the nature disclosed consisting in mixing sulfur-bearing fines with about 5-10% of plaster of Paris and then forming the resultant mixture into a multiplicity of blocks, and permitting the same to set prior to using the same. 55
35. A method of briquetting of the nature disclosed consisting in mixing a charge composed entirely of concentrates with about 5-10% of plaster of Paris and then forming the resultant mixture into a multiplicity of blocks, and permitting the same to set prior to using the same. 60
36. A method of briquetting of the nature disclosed consisting in mixing copper and sulfur-bearing fines with about 5-10% of plaster of Paris and then forming the resultant mixture into a multiplicity of blocks, and permitting the same to set prior to using the same. 65
37. A non-combustible, briquet of the nature disclosed adapted for the blast-furnace smelting of sulfur bearing ores and composed of a mass of comminuted pre-treated ore cemented together with a relatively small percentage of plaster of Paris. 70
38. A process of the nature disclosed consisting in subjecting a sulfur-bearing ore to a treatment adapted to evolve sulfur-bearing gases, converting gas so evolved into sulfuric acid, transforming a comminuted calcium compound into hydrated calcium sulfate by means of such acid, partially dehydrating such sulfate into plaster of Paris by means of the waste heat available from a metallurgical treatment of such ore, utilizing the resultant plaster of Paris as a binder in briquetting masses of finely divided ore, and then blast-furnace smelting the ore thus briquetted. 75
39. A process of the nature disclosed consisting in subjecting a sulfur-bearing ore to a treatment adapted to evolve sulfur-bearing gases, converting gas so evolved into sulfuric acid, transforming a comminuted calcium compound into hydrated calcium sulfate by means of such acid, partially dehy- 80
- 85
- 90
- 95
- 100
- 105
- 110
- 115
- 120
- 125
- 130

hydrating such sulfate into plaster of Paris, utilizing the resultant plaster of Paris as a binder in briquetting masses of finely divided ore, and then blast-furnace smelting the ore thus briqueted.

40. A process of the nature disclosed consisting in transforming a comminuted calcium compound into hydrated calcium sulfate by means of sulfuric acid, partially dehydrating such sulfate into plaster of Paris by means of the waste heat available from a metallurgical treatment of such ore, utilizing the resultant plaster of Paris as a binder in briquetting masses of finely divided ore, and then blast-furnace smelting the ore thus briqueted.

41. A process of the nature disclosed consisting in transforming a comminuted calcium compound into hydrated calcium sulfate by means of sulfuric acid, partially dehydrating such sulfate into plaster of Paris, utilizing the resultant plaster of Paris as a binder in briquetting masses of finely divided ore, and then blast-furnace smelting the ore thus briqueted.

42. A method of smelting a sulfur and

copper bearing material in which 20% of the sulfur content does not sufficiently exceed the copper content to yield a matte too low for economic converting, consisting in first briquetting the unroasted ore by means of a hydratable sulfur-bearing binder and then directly smelting such briquetted unroasted ore in a blast furnace.

43. A method of smelting a sulfur and copper bearing material in which 20% of the sulfur content does not sufficiently exceed the copper content to yield a matte too low for economic converting, consisting in first briquetting the unroasted ore by means of plaster of Paris and then directly smelting such briquetted unroasted ore in a blast furnace.

In witness whereof, I have signed the foregoing specification in the presence of the two subscribing witnesses at Santiago, Chili, this 23rd day of August, 1911.

BERNARD T. COLLEY.

Witnesses:

T. H. BARCLAY,  
J. F. MARTIN, Jr.